

Patented Oct. 23, 1923.

1,471,655

# UNITED STATES PATENT OFFICE.

FREDERICK J. GRIFFITHS AND DUKE N. A. BLACET, OF MASSILLON, OHIO.

## STEEL MANUFACTURE.

No Drawing.

Application filed December 31, 1920. Serial No. 434,397.

To all whom it may concern:

Be it known that we, FREDERICK J. GRIFFITHS and DUKE N. A. BLACET, citizens of the United States, and residents of Massillon, county of Stark, State of Ohio, have jointly invented a new and useful Improvement in Steel Manufacture, of which the following is a specification, the principle of the invention being herein explained and 10 the best mode in which we have contemplated applying that principle, so as to distinguish it from other inventions.

It is generally conceded that the presence of foreign substances in steel is injurious 15 thereto for the usual structural purposes to which steel is put; but for certain commercial uses where the steel is subjected to fatigue and vibratory stress we have found it desirable to impart to the steel a definite 20 fibrous structure. The purpose of the present invention accordingly is to secure this physical condition and control the occurrence of the same so that the fiber or grain of the steel will absorb the stress imposed 25 and thereby increase the endurance or fatigue properties of the metal.

To the accomplishment of the foregoing and related ends, the present invention consists of the steps hereinafter fully described 30 and particularly pointed out in the claims, the following description setting forth but one of several ways in which the principle of the invention may be embodied.

According to our present improved method, we deliberately and purposefully incorporate in the steel when originally cast, i. e., in the ingot, an ingredient or ingredients that will produce such fiber, striations or laminations in the resultant steel upon the subsequent working up of the ingot. Only relatively small proportions (one half of one per cent or less by weight) of such fiber producing ingredient need be introduced in order to have the effect indicated and as such ingredients, we may employ a variety of metallic, non-metallic or semi-metallic substances. Such substance should be finely ground or granular before it is introduced into the steel and as examples of suitable substance, we refer to ordinary furnace slag, brick dust and clay, any one of which, or combination thereof, will, upon subsequent

working of the steel produce well defined fibers or striations or laminations of the character desired.

The present improvement is equally applicable to ordinary carbon steel or to any of the so-called alloy steels wherein the presence of fiber is considered desirable. The substance employed to produce such fiber 55 can be mechanically introduced or thrown in the mold when the ingot is cast, or the dirt or other extraneous substances left on the stool, after casting and stripping an ingot, if simply allowed to remain in the mold when 60 the next ingot is cast, will serve the purpose as satisfactorily as the introduction of any of the particular ingredients named above. The amount of such ingredients, however, 65 can be better gaged when they are independently or separately introduced so as to produce the desired degree of fiber, which will of course vary, depending upon the 70 particular use to which the finishing steel is to be put.

Other forms may be employed embodying the features of our invention instead of the one here explained, change being made in the form of construction, provided the elements stated by any of the following claims or the 75 equivalent of such stated elements be employed, whether produced by our preferred method or by others embodying steps equivalent to those stated in the following claims.

We therefore particularly point out and 80 distinctly claim as our invention:—

1. In the manufacture of steel, the step which consists in introducing in the steel, while in molten condition, an ingredient that upon distribution throughout the mass 85 produces fiber-like striations, or laminations substantially as described.

2. In the manufacture of steel, the step which consists in introducing in the steel, while in molten condition, a finely-powdered or granular ingredient that upon distribution throughout the mass produces fiber-like striations, or laminations substantially 90 as described.

3. In the manufacture of steel, the step which consists in introducing in the steel, while in molten condition, finely-powdered or granular slag in relatively small quantity.

4. As a new product, a steel article having

defined striations or fibers or laminations produced by the presence therein of a relatively small quantity of a finely powdered or granular metallic, semi-metallic or non-metallic ingredient.

5. As a new product a steel article having defined striations or fibers or laminations

produced by the presence therein of a relatively small quantity of a finely powdered or granular slag.

10  
Signed by us, this 28th day of December, 1920.

FREDERICK J. GRIFFITHS.  
DUKE N. A. BLACET.